

Sept. 16, 1924.

1,508,861

A. TAUB

## PISTON

Filed March 8, 1922



**Inventor**

Fig. 2

By His Attorneys *Alex Taub*  
*Blockman, Spiegel & Bluest*

Patented Sept. 16, 1924.

1,508,861

# UNITED STATES PATENT OFFICE.

ALEX TAUB, OF DETROIT, MICHIGAN, ASSIGNOR TO GENERAL MOTORS CORPORATION, OF DETROIT, MICHIGAN, A CORPORATION OF DELAWARE.

## PISTON

Application filed March 8, 1922. Serial No. 542,038.

To all whom it may concern:

Be it known that I, ALEX TAUB, a citizen of the United States, and a resident of Detroit, county of Wayne, and State of Michigan, have invented certain new and useful Improvements in Pistons, of which the following is a full, clear, concise, and exact description, such as will enable others skilled in the art to which the invention relates to 10 make and use the same, reference being made therein to the accompanying drawings, which form a part of this specification.

The invention relates to pistons and more particularly to those of the type generally employed in connection with internal combustion engines.

The principal object of the invention is to provide a piston of soft metal, such as aluminum or one of its alloys, having different portions thereof capable of being formed integrally, as by casting, but of differing hardness.

It is common practice to utilize for the pistons of internal combustion engines a metal or alloy which is softer than the material of the cylinder walls, thereby reducing the wear of the cylinder to a minimum and preventing scoring of the walls. Since cast iron is commonly employed for the 30 cylinders, it is usual to form such pistons from a metal softer than cast iron, aluminum or one of its alloys being well recognized as suitable for that purpose because of its softness and other advantageous properties, including lightness.

Contact with the cylinder walls, however, occurs chiefly in the guide or skirt portion of the piston, in which region relative softness is of advantage as mentioned above; 40 whereas in the head portions of the piston and the region constituting a bearing for the wrist pin, a greater degree of hardness is desirable in order to avoid excessive wear in the pin bearings and piston ring grooves.

With the object therefore of producing a piston having a relatively soft skirt portion and a relatively hard head portion, at the same time retaining the advantages in simplicity, strength and cheapness of construction due to the formation of the piston in one piece, I propose to subject the piston to a treatment especially designed to develop different degrees of hardness in different portions thereof.

While various methods may be employed

to effect a variation in hardness between the head and skirt portions of the piston, I prefer to utilize a differential heat treatment and will describe herein a treatment which may be readily applied during the 60 casting of the piston. In accordance with this method, portions of the mold to be used in casting the piston may be formed of materials adapted to conduct heat rapidly from the surface of the molten metal, thereby chilling the metal which contacts with such portions of the mold and materially increasing the hardness in the chilled sections of the cast article.

The results, as well as one form of apparatus in which the operation may be carried out, are illustrated in the accompanying drawings, in which—

Fig. 1 is an elevation partly in cross-section representing a piston embodying the 75 invention; and

Fig. 2 is a cross-section representing a mold with a piston as cast therein.

Referring to the drawings, the piston represented in Fig. 1 includes a head portion 5 and skirt portion 6. Grooves 7, which may be formed in the process of casting, are provided in the head portion of the piston to receive the usual packing rings. Bearings 8, positioned intermediate the head and skirt portions, provide a means of support for the piston pin whereby the connecting rod may be attached to the piston. The head portion of the piston extending to approximately the plane of the axis of the piston pin bearings is hardened as indicated by the cross-hatching in order to resist wear. The piston pin bearings may also be hardened as indicated in Fig. 2. The hardening may be effected by the apparatus illustrated in Fig. 2, comprising outer mold members 10, 12, 12', and an inner mold member or core 11.

The lower portion of the outer mold is formed in sections 12, 12', to facilitate separation from the article after casting and may be of the character generally employed in die casting. The material from which these sections are formed may be iron or other material having good heat conducting 105 properties, while the upper portion 13 is of non-conducting material, such, for example, as ordinary molding sand. The inner mold member 11 is also of non-conducting material. The core 14 for the piston pin bearings 110

should also be of conducting material, as iron, in order to provide a chill for the bearing surfaces.

The cooling of the head portion of the piston may be facilitated by providing a hollow space 15 within the portions 12, 12', of the mold, in which space a cooling fluid, as steam, may be caused to circulate, suitable supply and outlet passages being provided 10 as indicated at 16, 17, respectively.

In casting pistons in apparatus such as described, it will be understood that the portions which are cast in contact with the conducting surfaces of the parts 12, 12', 14, will 15 be chilled and thereby rendered harder than the portions which are cast in contact with the non-conducting materials. In accordance with this process it has been found possible to produce an alloy piston the skirt 20 portion of which has a hardness, as represented on the Brinell scale, of 85 to 95, while the head portion has a hardness of 125 to 140.

It will be understood that the details of 25 structure and operation may be varied widely without departing from the spirit and scope of the invention, and therefore I do not wish to be limited to the specific details above set forth except as required by

the language of the appended claims in view 20 of the prior art.

I claim:

1. A piston formed in one piece from metal softer than cast iron and having the head portion harder than the skirt portion. 35

2. A piston formed in one piece from metal comprising chiefly aluminum, the head portion of the piston being harder than the skirt portion.

3. A piston formed in one piece from 40 metal softer than cast iron and having the portions adjacent to the piston ring grooves hardened to resist wear, the skirt portion being softer than the said hardened portion.

4. A piston formed in one piece from 45 metal softer than cast iron and having the portions adjacent to the piston ring grooves and to the piston pin bearings hardened to resist wear, the skirt portion being softer than the said hardened portion. 50

5. A cast metal piston formed in a single piece from metal comprising chiefly aluminum, the portions adjacent to the head, ring grooves and pin bearings being chilled to resist wear and the skirt portion being softer than the said chilled portions. 55

In testimony whereof I affix my signature.  
ALEX TAUB.